

1

3,764,262

## PROCESS FOR THE DYEING AND PRINTING OF TEXTILE MATERIALS

Dietrich Hildebrand, Odenthal, and Helmut Kirschnek, Leverkusen-Schlebusch, Germany, assignors to Bayer Aktiengesellschaft, Leverkusen, Germany  
 No Drawing. Filed Sept. 8, 1970, Ser. No. 70,514  
 Claims priority, application Germany, Sept. 11, 1969,  
 P 19 45 965.5  
 Int. Cl. D06p 1/68, 1/84

U.S. Cl. 8—84

12 Claims

### ABSTRACT OF THE DISCLOSURE

The invention relates to the dyeing and printing of textile materials with chlorinated hydrocarbon/water dyestuff emulsions, the aqueous phase of which contains a solution of water-soluble dyestuffs and the chlorinated hydrocarbon phase of which may be a solution of dyestuffs soluble in chlorinated hydrocarbons, and to an after-treatment in chlorinated hydrocarbon solutions containing compounds which are interface-active in chlorinated hydrocarbons.

The invention relates to a process for the dyeing and printing of textile materials with chlorinated hydrocarbon/water dyestuff emulsions; the process is characterised in that the textile materials are dyed or printed with chlorinated hydrocarbon/water dyestuff emulsions the aqueous phase of which is a solution of water-soluble dyestuffs and the chlorinated hydrocarbon phase of which may be a solution of dyestuffs soluble in chlorinated hydrocarbons; and that the materials are subsequently, possibly after a heat treatment, subjected to an after-treatment in chlorinated hydrocarbon solutions containing compounds which are interface-active in chlorinated hydrocarbons and convert the dyestuffs used into a form soluble or dispersible in chlorinated hydrocarbons.

The compounds are expediently used in an amount of 0.02–2 percent by weight, referred to the weight of the chlorinated hydrocarbons.

The compounds which are used in the chlorinated hydrocarbon baths for after-treatment according to the invention, in order to convert the dyestuffs used into a form soluble or dispersible in chlorinated hydrocarbons, can be divided into two groups, on account of their behaviour towards the various dyestuffs.

Group (A): This group comprises the compounds which convert basic dyestuffs as well as acidic dyestuffs, anionic metal complex dyestuffs which are free from sulpho groups, or reactive dyestuffs which contain sulpho groups, into a form soluble or dispersible in chlorinated hydrocarbons.

Because of their universal applicability, the compounds of this group are preferably used in the after-treatment baths of the process according to the invention.

Group (B): This group comprises the compounds which convert only basic dyestuffs into a form soluble or dispersible in chlorinated hydrocarbons.

It is a precondition for the usability of the compounds of both groups that they should be soluble in the chlorinated hydrocarbons in the concentrations in which they are used at temperatures below 50° C.

The compounds belonging to group (A) are the following:

#### (1) Onium compounds of the formulae



2

in which

A denotes a nitrogen or phosphorus atom;  
 R<sub>1</sub> stands for an alkyl, alkenyl or aralkyl radical which carries 12–18 carbon atoms and may be interrupted by hetero atoms such as oxygen, sulphur and/or nitrogen atoms;

R<sub>2</sub> and R<sub>3</sub>, independently of one another, denote an alkyl, alkenyl or aralkyl radical which carries 1–28 carbon atoms and may be interrupted by hetero atoms such as oxygen, sulphur and/or nitrogen atoms; and may be substituted;

R<sub>4</sub> means an optionally substituted C<sub>1</sub>–C<sub>14</sub>-alkyl, C<sub>1</sub>–C<sub>14</sub>-alkenyl, cycloalkyl or aralkyl radical, or together with R<sub>3</sub> forms a non-aromatic 5- or 6-membered heterocycle, with the proviso that the sum total of the carbon atoms contained in R<sub>1</sub>, R<sub>2</sub>, R<sub>3</sub>, and R<sub>4</sub> amounts to at least 20 and at most 60; and X<sup>−</sup> denotes an anion.

(2) Quaternary ammonium compounds of the formula



in which

R<sub>1</sub>, R<sub>3</sub> and R<sub>4</sub> have the same meaning as in the Formulae I and II; and

Z stands for an alkylene radical which contains 1–8 carbon atoms and may be interrupted by hetero atoms such as oxygen atoms, or denotes a 1,4-bis-methylene-benzene radical, with the proviso that the sum total of the carbon atoms contained in R<sub>1</sub>, R<sub>3</sub>, R<sub>4</sub> and Z amounts to at least 20 and at most 60; and

Y<sup>−</sup> is an anionic grouping such as —SO<sub>3</sub><sup>−</sup>, —OSO<sub>3</sub><sup>−</sup>, —SO—SO<sub>3</sub><sup>−</sup>, —O—PO<sub>3</sub><sup>−</sup> or —COO<sup>−</sup>.

(3) Amines of the formula



in which

R<sub>1</sub> and R<sub>4</sub> have the same meaning as in the Formulae I and II; and

R<sub>5</sub> stands for hydrogen or R<sub>3</sub> where R<sub>3</sub> has the same meaning as in Formula I, or together with R<sub>4</sub> forms a 5- or 6-membered non-aromatic heterocycle, with the proviso that the sum total of the carbon atoms contained in R<sub>1</sub>, R<sub>4</sub> and R<sub>5</sub> amounts to at least 20 and at most 60.

(4) Aminoxides of the formula



in which

R<sub>1</sub>, R<sub>3</sub> and R<sub>4</sub> have the same meaning as in the Formulae I and II, with the proviso that the sum total of the carbon atoms contained in R<sub>1</sub>, R<sub>3</sub> and R<sub>4</sub> amounts to at least 20 and at most 60.

R<sub>1</sub>: Suitable alkyl, alkenyl or aralkyl radicals which contain 12–28 carbon atoms and may be interrupted by hetero atoms such as oxygen, sulphur and/or nitrogen atoms are the following, for example:

C<sub>12</sub>–C<sub>28</sub>-alkyl radicals, such as the dodecyl, tetradecyl, hexadecyl, octadecyl, eicosyl, docosyl, 3,6,9-trimethylhexadecyl, 1-octyl-dodecyl and 1-undecyl-dodecyl radicals;

Saturated radicals with a carbon chain interrupted by hetero atoms, such as 3-oxa-nonadecyl-(1), 3-oxa-heneicosyl-(1), 4-oxa-docosyl-(1), 3,6-dioxa-docosyl-(1), 3-thia-heneicosyl-(1), dodecyl-aminoethyl, hexadecylaminopropyl, octadecyl-aminoethyl, octadecyl-aminopropyl, octadecyl-aminobutyl, eicosyl-aminopropyl, docosyl-aminopropyl radical and especially the dodecanoyl-aminoethyl, tetradecanoyl-aminoethyl, hexadecanoyl-aminobutyl, octadecanoyl-aminopropyl, eicosanoyl-aminopropyl and docosanoyl-aminoethyl radicals;

$C_{12}$ - $C_{28}$ -alkenyl radicals such as the oleyl, linolyl, linolenyl, eicosenyl, docosenyl and 2-ethyl-octadecen-9,10-yl-(1)-radicals;

Unsaturated radicals with a carbon chain interrupted by hetero atoms, such as 3-oxa-nonadecen-10,11-yl-(1), 4-oxadocosen-13,14-yl-(1), hexadecen-7,8-yl-aminoethyl, octadecen-9,10-yl-aminoethyl, docos-13,14-yl-aminopropyl and especially the oleoyl-aminoethyl, linolenoyl-aminopropyl, linolenoyl-aminoethyl, eicosenoyl-aminopentyl and docosenoyl-aminoethyl radicals;

Aralkyl radicals with a carbon chain interrupted by hetero atoms such as the (4-nonyl-phenyl)-ethyl-carboxyethyl radical.

$R_2$  and  $R_3$ : Suitable alkyl, alkenyl or aralkyl radicals which contain 1-28 carbon atoms and may be interrupted by hetero atoms and/or may be substituted, are the following, for example:

$C_1$ - $C_{28}$ -alkyl radicals such as the methyl, ethyl, isopropyl, dodecyl, hexadecyl, octadecyl, eicosyl and docosyl radicals;

$C_1$ - $C_{28}$ -alkenyl radicals such as the buten-3,4-yl-(1)- and undecen-10,11-yl-(1) radicals;

Substituted alkyl and alkenyl radicals such as the 2-hydroxyethyl, 3-hydroxypropyl, 3-hydroxybutyl, 13-hydroxy-octadecen-9,10-yl-(1), 2-chloroethyl, 3-chloropropyl, 11-bromoundecyl, 13-chlorotadecen-9,10-yl-(1)-13,14-dichlorodocosyl, 2-cyanoethyl, 3-cyanopropyl, 11-cyano-undecyl, 3-aminopropyl, 3-(N-methyl-amino)-butyl, 11-amino-undecyl, 13-(N-methylamino)-docosyl and the carbothoxy-ethyl radicals;

Alkyl and alkenyl radicals with a carbon chain interrupted by hetero atoms, such as the methoxy-ethyl, ethoxy-butyl, 3-oxa-dodecyl-(1), 3-oxa-heneicosyl-(1)-3,6-dioxa-docosyl-(1), 4-thia-hexenyl-(1), 3-thia-pentadecyl-(1), N-methyl-2-aminoethyl, N-ethyl-3-aminopropyl, N-propyl-3-aminopropyl, N-dodecyl-2-aminoethyl, N-octadecyl-3-aminopropyl, N-heneicosyl-4-aminobutyl and the N-docosyl-6-aminobutyl radicals;

Aralkyl radicals such as the benzyl, 4-chlorobenzyl, 3-methyl-benzyl and 4-nonylphenyl-ethyl-carboxyethyl radicals.

$R_4$ : Suitable, optionally substituted  $C_1$ - $C_{14}$ -alkyl,  $C_1$ - $C_{14}$ -alkenyl, cycloalkyl or aralkyl radicals are the following, for example:

$C_1$ - $C_{14}$ -alkyl radicals such as the methyl, ethyl, isopropyl, sec.-butyl, 2-ethylhexyl, dodecyl, 2-hydroxyethyl, 3-hydroxy-propyl, 2-methoxyethyl, 2,3-epoxypropyl, chloromethyl, 2-bromoethyl, chloropropyl, 2-hydroxy-3-chloropropyl, 2,3-epoxy-propyl, carbothoxymethyl, carboxamidomethyl, 2-cyanoethyl, acetoxyethyl and 3-trimethylammonium-propyl radicals.

60

$C_1$ - $C_{14}$ -alkenyl radicals such as the buten-3,4-yl-(1)-undecen-10,11-yl-(1) radicals;

Cycloalkyl radicals such as the cyclohexyl, 4-methylcyclohexyl, 3-octylcyclohexyl and 4-chlorocyclohexyl radicals;

Aralkyl radicals such as the benzyl, 3-methylbenzyl, 4-cyclohexyl-benzyl, 4-methoxybenzyl and 3-chlorobenzyl radicals.

Suitable 5- or 6-membered heterocycles which may be formed by  $R_4$  together with  $R_3$ , are primarily the morpholine and piperidine rings.

Suitable anions  $X^-$ , are anions of organic acids, such as the chloride, bromide, iodide and sulphate ions; the anions of acidic esters of inorganic acids, such as the methyl-sulphate, ethyl-sulphate and toluene-sulphate ions; and the anions of organic acids, such as the acetate, propionate, ethyl-caproate, oleate, behenate, benzoate and salicylate ions.

Z: Suitable alkylene radicals which contain 1-8 carbon atoms and may be interrupted by hetero atoms are the following, for example:

Alkylene radicals, such as the methylene, ethylene, propylene-1,2, propylene-1,3, butylene and hexylene radicals;

Alkylene radicals interrupted by hetero atoms, such as the 3-oxa-hexylene-1,6 and 3,6-dioxa-octylene-1,8 radicals.

Representatives of the onium compounds of the Formula I are the following, for example:

- 30 (a) Ammonium compounds, such as  
 dodecyl-dimethyl-benzyl ammonium chloride  
 docosyl-dimethyl-benzyl ammonium chloride  
 oleyl-trimethyl ammonium chloride  
 distearyl-dimethyl ammonium chloride  
 dioleyl-dimethyl ammonium chloride  
 lauryl-dimethyl-2-chloroethyl ammonium chloride  
 dilauryl-bis-2-chloroethyl ammonium chloride  
 lauryl-dimethyl-hydroxyethyl ammonium chloride  
 dodecyl-dimethyl-vinyl ammonium chloride  
 lauryl-methyl morpholinium chloride  
 stearyl-di-(hydroxydiethoxyethyl)-benzyl ammonium bromide  
 oleyl-di-[(5-hydroxy)-3-oxa-pentyl-(1)]-ammonium chloride  
 45 coconut-di-[(8-hydroxy)-3,6-dioxa-octyl-(1)]-benzyl ammonium chloride  
 coconut-dimethyl-benzyl ammonium chloride  
 coconut-dimethyl- $\gamma$ -hydroxypropyl ammonium chloride  
 di-hexadecyl-methyl-benzyl ammonium chloride  
 50 di-octadecyl-dimethyl ammonium chloride  
 di-octadecyl-ethyl-methyl ammonium ethylsulphate  
 di-docosyl-dimethyl ammonium chloride  
 di-eicosyl-dimethyl ammonium bromide  
 55 1-( $\beta$ -octadecyl-aminoethyl)-2-octadecyl-3-methyl imidazolinium chloride  
 and the compounds of the formula





(b) Phosphonium compounds such as

dodecyl-dimethyl-benzyl phosphonium chloride  
 tetradecyl-dimethyl-benzyl phosphonium chloride  
 octadecyl-trimethyl phosphonium chloride  
 octadecyl-dimethyl-hydroxyethyl phosphonium chloride  
 oleyl-dimethyl-benzyl phosphonium chloride.

Representatives of the onium compounds of the Formula II are the following sulphonium compounds, for example:

bis-dodecyl-methyl sulphonium methylsulphate  
 behenyl-dimethyl sulphonium chloride  
 oleyl-methyl-benzyl sulphonium chloride.

Representatives of the quaternary ammonium compounds of the Formula III are the following, for example: 51



Representatives of the amines of the Formula IV are the following, for example:

60 N-methyl-N-2-hydroxyethyl-N-[ $\gamma$ -(octadecanoyl)-amino]-propyl]-amine  
 N,N-dimethyl-4-dodecyl-aniline  
 N-octadecyl-piperidine

65 1-( $\beta$ -hydroxyethyl)-2-octadecyl-imidazoline  
 1-( $\beta$ -octadecanoylaminoethyl)-2-octadecyl-imidazoline  
 N-oleyl-N',N'-diethyl-ethylene-diamine  
 N-oleyl-N',N'-dimethyl-propylene-diamine-(1,3)  
 N-oleyl-N',N'-diethyl-propylene-diamine-(1,3)

70 N-[1-(undecyl)dodecyl]-N,N-dimethylamine





Representatives of the aminoxides of the Formula V are the following, for example:

N,N-dibutyl-N-dodecyl-aminoxide  
 N,N-dimethyl-N-(3-octadecanoylamino-propyl)-aminoxide  
 N,N-dimethyl-N-[3-(N'-octadecyl-carbamanyl)-amino-propyl]-aminoxide  
 N,N-dimethyl-N-(3-octadecylsulphonylamino-propyl)-aminoxide  
 N,N-dimethyl-N-(3-oleoylamino-propyl)-aminoxide  
 N-methyl-N,N-bis-[3-(octadecanoylamino)-propyl]-aminoxide  
 N-methyl-N,N-bis-[3-(dodecanoylamino)-propyl]-aminoxide  
 N-methyl-N-β-cyanoethyl-N-[3-(octadecanoylamino)-propyl]-aminoxide  
 N-methyl-N-β-hydroxyethyl-N-[3-oleoylamino)-propyl]-aminoxide  
 N-methyl-N-[3-(octadecanoylamino)-propyl]-N-[β-(octadecanoyloxy)-ethyl]-aminoxide  
 N,N-dimethyl-N-[β-(N'-octadecylcarbamanyl)-hydroxyethyl]-aminoxide  
 N-methyl-N-benzyl-N-dodecylaminoxide  
 N,N-dimethyl-N-(4-dodecyl-phenyl)-aminoxide  
 N-1-(β-hydroxyethyl)-2-octadecyl-imidazoline-N-oxide  
 1-(β-octadecanoylamino-ethyl)-2-octadecyl-imidazoline-N-oxide  
 N,N-diethyl-N'-methyl-N'-octadecyl-ethylene-diamine-N,N'-dioxide  
 N,N,N',N'-tris-(β-hydroxyethyl)-N'-octadecyl-1,3-propylene-diamine-N,N'-dioxide  
 N,N,N',N'-tetramethyl-aminomethyl-stearylamine-N,N'-dioxide  
 N,N-dimethyl-N-3,6,9-trioxa-heneicosyl-aminoxide  
 N,N-dimethyl-N-4,7,10,13,16-penta-oxa-19-thia-hentriacetyl-aminoxide  
 N-monoxides of the reaction products of 3-30 mol ethylene oxide on 1 mol eicosylamine, furthermore  
 N-methyl-N-octadecyl-N-[3-(di-β-chloroethylamino)-propyl]-aminoxide  
 N-methyl-N-octadecyl-N-(3-dimethylamino)-propyl-aminoxide  
 N-methyl-N-octadecyl-N-[3-(γ-aminopropylamino)-propyl]-aminoxide.

The compounds belonging to the group (B) are the following:

(1) Acidic sulphuric acid and phosphoric acid esters or their alkali metal, alkaline earth metal or ammonium salts containing at least one hydrocarbon radical which carries 16 carbon atoms, e.g.

Sulphates of mono- and polyhydric alcohols containing at least 16 carbon atoms, such as cetyl sulphate, stearyl sulphate, oleyl sulphate, behenyl sulphate, 2-hexyl-decanol-1-sulphate, 2,4,6-triethyl-decanol-1-sulphate, 3,10-diethyl-tridecanol-7-sulphate, 1,2-diundecyl-ethylene-glycol monosulphate, glycerol-monostearate monosulphate;

The sulphates obtainable by sulphonation of unsatu-

rated fatty acids, fatty acid esters and fatty acid ester amides, such as oleic acid sulphate, oleic acid butyl ester sulphate, ricinoleic acid ethyl ester sulphate, oleic acid ethylamide sulphate, oleic acid ethanolamide sulphate, oleic acid diisobutylamide sulphate, oleic acid anilide sulphate,



Sulphates of acylated or alkylated polyglycol ethers containing not more than 30 ethylene oxide and/or 80 propylene oxide units in the molecule, such as

hexadecyl diglycol ether sulphate  
 octadecyl tetraglycol ether sulphate  
 octadecenyl octaglycol ether sulphate  
 hexadecanoyl diglycol ether sulphate  
 octadecanoyl tetraglycol ether sulphate  
 dodecylphenol diglycol ether sulphate  
 octadecyl tetrapropylene glycol ether sulphate  
 25 dodecylphenol-tripropylene glycol ether sulphate  
 $\text{CH}_3-(\text{CH}_2)_7\text{CH}=\text{CH}-(\text{CH}_2)_7\text{CONH-}(\text{C}_2\text{H}_4\text{O})_{16}\text{SO}_3\text{Na}$   
 polypropylene glycol ether monosulphate (mol. weight 30 4000)

Sulphates of acylated or alkylated alkanolamines, such as N-acetyl-oleylamine sulphate



Sulphates of monohydroxy-polycarboxylic acid esters, such as



Acidic phosphoric acid esters, such as dioctadecyl phosphate and



(2) Aliphatic, araliphatic and aromatic sulphonic acids 50 or their alkali metal, alkaline earth metal or ammonium salts containing at least one hydrocarbon radical which carries 16 carbon atoms, e.g.

Alkyl-sulphonic acids, such as



Substituted aliphatic sulphonic acids, such as





## 11

should also contain 0.001-8 percent by weight, referred to the weight of the chlorinated hydrocarbons, of water-miscible organic solvents, such as isopropanol, benzyl alcohol, phenoxy-ethanol, acetonitrile, hydroxypropionitrile, dimethyl sulphoxide, dimethyl formamide or methyl glycol acetate; and to add to the chlorinated hydrocarbon after-treatment baths 0.01-0.5 percent by weight, referred to the weight of the chlorinated hydrocarbons, of acetic acid when after-treating dyeings and prints obtained with cationic dyestuffs, and 0.01-0.5 percent by weight, referred to the weight of the chlorinated hydrocarbons, of mono-, di- or triethanolamine and/or 0.01-1 percent by weight, referred to the weight of the chlorinated hydrocarbons, of acetic acid when after treating dyeings or prints obtained with acidic dyestuffs, anionic sulpho group-free metal complex dyestuffs and sulpho group-containing reactive dyestuffs.

The process according to the invention is suitable for the dyeing with cationic dyestuffs as well as for the dyeing with acid dyestuffs, anionic, sulpho group-free metal complex dyestuffs and sulpho group-containing reactive dyestuffs.

Suitable cationic dyestuffs are methine, azomethine, hydrazone, azacyanine, triarylmethane, xanthene, thioxanthene, acridine, oxazine, thiazine and phenazine dyestuffs; furthermore, the basic dyestuffs of the azo, anthraquinone or phthalocyanine series, such as are described e.g. in Colour Index, vol. I, 2nd Edition (1956), pages 1617-1654, and in the Supplement of 1963, and also in French patent specification No. 1,480,930.

Suitable acid dyestuffs are all water-soluble dyestuffs of the azo, anthraquinone, triphenyl-methane and phthalocyanine series which contain up to four sulpho groups; examples of anionic sulpho group-free metal complex dyestuffs are the sulpho group-free 1:2 metal complex dyestuffs of the azo and triphenylmethane series which contain at least two groups capable of dissociation; and the sulpho group-containing reactive dyestuffs comprise e.g. water-soluble dyestuffs of the azo, anthraquinone and phthalocyanine series, which contain at least one fibre-reactive group, for example, a monochloro-triazinyl, dichlorotriazinyl, dichloro-quinoxalinyl, trichloro-pyrimidinyl, difluoro-chloro-pyrimidinyl,  $\alpha$ -bromoacrylamide group or the  $\beta$ -hydroxyethyl-sulphuric acid semi ester group.

Insofar as thickening agents are required for preparing the dyestuff emulsions, thickening agents poor in body are preferred for the process according to the invention.

The process according to the invention is suitable for the dyeing and printing of all textile materials which can be dyed or printed with the aforesaid dyestuffs. These include, for example, the textile materials of polyacrylonitrile, polyester, cellulose 2½-acetate, cellulose triacetate, synthetic polyamides and silk, which can be dyed with basic dyestuffs; the textile materials of natural or regenerated cellulose such as cotton, staple fibre and rayon, cellulose 2½-acetate, cellulose triacetate, of natural polyamides such as wool and silk, and of synthetic polyamides such as polyhexamethylene diamine adipate, polycaprolactam or poly- $\alpha$ -aminoundecanoic acid, which can be dyed with acid, metal complex and reactive dyestuffs. The present process has proved particularly satisfactory for the dyeing and printing of mixtures of these types of fibres, e.g. mixtures of polyacrylonitrile/staple fibre, polyester/cotton, polyester/staple fibre, polyamide/staple fibre, polyamide/cotton, cellulose 2½-acetate/staple fibre, cellulose triacetate/staple fibre or polyacrylonitrile/polyester.

The textile materials may be present in various stages of processing, e.g. as threads, ribbons, combed material, yarn, fabrics, knitted fabrics or ready-made goods.

The chlorinated hydrocarbons expediently used in the after-treatment baths of the process according to the invention are aliphatic chlorinated hydrocarbons, such as methylene chloride, chloroform, carbon tetrachloride,

## 12

1,1 - dichloroethane, 1,2 - dichloroethane, 1,1,1-trichloroethane, 1,1,2 - trichloroethane, 1,1,1,2 - tetrachloroethane, 1,1,2,2 - tetrachloroethane, pentachloroethane, 1-chloropropane, 1,2 - dichloropropane, 1-chlorobutane, 2-chlorobutane, 1,4 - dichlorobutane, 1 - chloro - 2 - methyl-propane, 2 - chloro - 2 - methyl - propane or 4 - chloro-2-methyl-propane. Tetrachloroethylene, trichloroethylene and 1,1,1 - trichloropropane have proved particularly satisfactory.

The process according to the invention is carried out by applying the dyestuffs to the textile materials by means of the dyestuff emulsions according to the exhaust, spray, padding or printing process at temperatures from 20 to 120° C. Subsequently, possibly after a conventional heat treatment such as drying, steaming or thermosolising, the textile materials are subjected in a continuous or discontinuous operation to an after-treatment in chlorinated hydrocarbon solutions containing interface-active compounds which convert the dyestuffs used into a form soluble or dispersible in chlorinated hydrocarbons. Optionally, this after-treatment is followed by rinsing in pure chlorinated hydrocarbon. By this after-treatment any non-fixed dyestuffs or dyeing auxiliaries are so completely removed from the textile materials that, after separation of the wash liquor and removal of the last solvent residues by blowing out with air or steam, the materials can be stored without any further after-treatment.

The emulsions to be used as dyebaths or printing pastes may either contain water as a continuous phase and the chlorinated hydrocarbons as a discontinuous phase, or they may contain the chlorinated hydrocarbons as a continuous phase and water as a discontinuous phase. In any case the aqueous phase is a solution of water-soluble dyestuffs; the chlorinated hydrocarbon phase may be a solution of a dyestuff soluble in chlorinated hydrocarbons, but it may also be formed by chlorinated hydrocarbons free from dyestuff.

The amounts of dyestuff dissolved in the respective phases depend upon the desired depth of colour of the dyeings or prints, upon the solubility of the dyestuffs, and upon whether the exhaust, spray, padding or printing process is applied. In general, amounts of 0.2 to 50 g. of dyestuff per litre of dyestuff emulsion have proved satisfactory.

As emulsifiers for preparing the dyestuff emulsions, there may be used the compounds which usually serve for preparing oil-in-water and water-in-oil emulsions. Non-ionic emulsifiers have proved especially satisfactory for the process according to the invention.

Suitable non-ionic emulsifiers are the commercial non-ionic emulsifiers, for example, reaction products of 1 mol of fatty alcohols, fatty acids, fatty amines, fatty acid amides, fatty acid alkanolamides, fatty acid glycerides, alkyl-phenols, alkyl-benzyl-phenols, alkyl-aryl-benzyl-phenols, aryl-styryl-phenols or abietic acid, with 1-100 mol ethylene oxide; furthermore, fatty acid esters of aliphatic polyhydroxy compounds and fatty acid alkanolamides.

The amounts of emulsifier required for preparing and stabilising the emulsions should not exceed 10 percent by weight, referred to the weight of the emulsions, and should preferably amount to 0.2 to 5 percent by weight.

Besides the dyestuffs and emulsifiers, the dyestuff emulsions may contain the usual dyeing auxiliaries, e.g. urea. The amounts of these auxiliaries depend on the dyestuffs used and on the dyeing process. In general, they amount to about 10 to 500 percent by weight, referred to the weight of the dyestuffs.

The emulsions can be prepared in the usual way. It has proved expedient to prepare the solutions forming the two phases separately and to emulsify, after the addition of the emulsifiers, with the aid of rapid stirrers or turbomixers.

Chlorinated hydrocarbons which can serve for the preparation of the dyestuff emulsions are those chlorinated

hydrocarbons which are also suitable for the after-treatment baths. Tetrachloroethylene, trichloroethylene and 1,1,1-trichloropropane have proved especially satisfactory also in the dyestuff emulsions.

With the aid of the process according to the invention it is possible to dye textile materials of various kinds with the conventional fastness properties in a gentle and practical way without the occurrence of waste water. The process according to the invention combines the advantages of dyeing from aqueous media (use of conventional dyestuffs, good fastness properties of the resultant dyeings) with the advantages of dyeing from organic solvents (unimpaired appearance of the goods, virtually no occurrence of waste water), without having the disadvantages of these processes.

A particular advantage of the process according to the invention consists in that textile materials can be dyed in the chlorinated hydrocarbon medium in a single bath with water-soluble dyestuffs and with dyestuffs soluble in chlorinated hydrocarbons.

The process according to the invention is therefore eminently suitable for the dyeing and printing of materials of cellulose fibres and of mixtures thereof with synthetic fibres with the use of water-soluble reactive dyestuffs for the cellulose fibre component and of disperse dyestuffs soluble in chlorinated hydrocarbons for the synthetic fibre component, and well as for the dyeing and printing of polyacrylonitrile/polyester fibre mixtures with the use of cationic water-soluble dyestuffs for the polyacrylonitrile component and of disperse dyestuffs for the polyester fibre component.

From Belgian patent specification No. 707,187 there is known a process for the dyeing of textile materials from chlorinated hydrocarbons, in which the textile materials are dyed in chlorinated hydrocarbon/water emulsions containing water-soluble or water-dispersible dyestuffs in the aqueous phase. If this process is used for dyeing with water-soluble dyestuffs, especially reactive dyestuffs and cationic dyestuffs, then dyeings of unsatisfactory fastness to wet processing are obtained, since the proportion of dyestuff which is not bound by the fibre is only incompletely removed by the subsequent washing of the dyeings with chlorinated hydrocarbons. To achieve satisfactory fastness to wet processing, the dyeings must therefore be rinsed with aqueous liquors. By using aqueous wash liquors, however, the advantages of dyeing from organic solvents (unimpaired appearance of the goods, slight occurrence of waste water) are cancelled out.

Compared with the process of the Belgian patent specification, the process according to the invention has not only the advantage of permitting dyeing with water-soluble dyestuffs and with dyestuffs soluble in chlorinated hydrocarbons from chlorinated hydrocarbon/water emulsions; it has primarily the advantage that, due to the after-treatment with the chlorinated hydrocarbon solutions containing compounds which convert the dyestuffs into a form soluble or dispersible in chlorinated hydrocarbons, dyeing with water-soluble dyestuffs, e.g. reactive dyestuffs and cationic dyestuffs, without having recourse to aqueous baths, yields dyeings of the same good fastness to wet processing as is achieved when dyeing from aqueous baths.

The parts given in the following examples are parts by weight; the constitution of the dyestuffs market with the figures (I)-(XVIII) are given in the table following the examples.

#### EXAMPLE 1

A polyester/cotton mixed fabric (65:35) is padded with an emulsion consisting of

15 parts of the dyestuff XVI

2 parts nonylphenol pentadecaethylene glycol ether

1 part oleic acid ethanolamide

20 parts of the dyestuff XIII

60 parts urea  
8 parts sodium bicarbonate  
94 parts of water and  
800 parts perchloroethylene

5 (liquor absorption 80%), dried at 80° C. for 1 minute and thermosolised at 180° C. for 30 seconds.

The fabric then passes, with a time of residence of 1.5 minutes each time, through four successive closed washing aggregates which operate according to the counter-current principle and contain a solution at 55° C. which consists of

4 parts of the compound of the formula



15 1 part of water  
20 5 parts of 30% acetic acid and  
990 parts perchloroethylene

and is mechanically agitated. The liquor ratio for this after-treatment amounts to 1:50. After mechanical separation of the rinsing liquor by squeezing, the fabric is freed from the adhering solvent residues by blowing with hot air, and stored. A clear yellow/red bicolour dyeing of good fastness properties is obtained. No waste water occurs in the after-treatment.

If the after-treatment is carried out by the same method with perchloroethylene without the additives according to the invention, then the non-fixed dyestuff component which is insoluble in perchloroethylene is not removed from the fabric, and the fastness properties of the resultant dyeing are therefore unsatisfactory.

If the after-treatment according to the invention described above is retained with the difference that the dyestuffs are not applied from the chlorinated hydrocarbon/water emulsion described above but from a pure aqueous dyebath in which the dyestuff XIII is dissolved but the dyestuff XVI is present in disperse form with the aid of dispersing agents, then a less clear yellow/red bicolour dyeing is obtained.

If the 5 parts of the compound of the formula



45 50 are replaced with 5 parts of one of the compounds of the Formulae (a)-(l)





or with 5 parts of a mixture of  
2.5 parts of the compound of the formula



and  
2.5 parts isopropanol

or with 5 parts of a mixture of the compounds (a)–(l),  
then an equally good after-treatment effect is achieved.

#### EXAMPLE 2

A polyester/polyacrylonitrile mixed fabric (50:50) is padded with an emulsion consisting of

20 parts of the dyestuff I  
10 parts of the dyestuff XVI  
4 parts methyl glycol acetate  
4 parts glycerol monoacetate  
1 part oleic acid ethanolamide  
3 parts nonylphenol decaethylene glycol ether  
10 parts of 60% acetic acid  
148 parts of water and  
800 parts perchloroethylene

(liquor absorption 80%) and thermosolised at 180° C. for 1 minute.

Subsequently, the fabric web successively passes, in a liquor ratio of 1:50 and with a time of residence of 2 minutes each time, through four solutions of

5 parts sodium dodecyl-benzene sulphonate  
0.5 part of 60% acetic acid and  
5 parts of water in 989.5 parts perchloroethylene

which have been heated to 50° C. and are mechanically agitated, and subsequently, with a time of residence of 1 minute, through a rinsing bath of pure perchloroethylene which has been heated to 50° C. After separating the rinsing liquor, the fabric is freed from the adhering perchloroethylene by blowing with air. The resultant yellow dyeing is rinsed clear without the occurrence of waste water and has the same fastness properties as a dyeing after-treated with an aqueous liquor.

If the after-treatment is carried out by the same method with perchloroethylene without the additives according to

the invention, then the non-fixed, perchloroethylene-insoluble dyestuff is not removed from the fabric and the fastness properties of the resultant dyeing are therefore unsatisfactory.

If the 5 parts sodium dodecyl-benzene sulphonate are replaced with

5 parts dodecyl-benzene-sulphonic acid or

5 parts sodium diisobutyl-naphthalene-sulphonate or

5 parts sodium C<sub>16</sub>-paraffin sulphonate or

5 parts of the compound of the formula



or

5 parts of a 1:1 mixture of sulphonated sperm oil and sulphonated olive oil or

5 parts of the compound of the formula



or

7 parts of a mixture of 5 parts of the compound of the formula



and 2 parts oleyl alcohol heptadecaethylene glycol ether,

then an equally well-rinsed dyeing is obtained.

An equally satisfactory dyeing is also obtained when the 989.5 parts perchloroethylene are replaced with the same amount of 1,1,1-trichloroethane.

#### EXAMPLE 3

A polyacrylonitrile fabric is padded with an emulsion consisting of

20 parts of the dyestuff II

2 parts oleyl alcohol eicosoethylene glycol ether

12 parts β-cyanoethyl formamide

4 parts nonylphenol decaethylene glycol ether

10 parts of 60% acetic acid,

100 parts of water and

852 parts perchloroethylene,

(liquor absorption 100%), dried at 110° C. for 1 minute and steamed at 102° C. for 15 minutes.

The fabric is then treated in a liquor ratio of 1:100 in a bath consisting of

10 parts of the compound of the formula



10 parts of water and

980 parts perchloroethylene

at 55° C. for 6 minutes, subsequently rinsed twice with fresh perchloroethylene and, after separating the liquor, freed from the perchloroethylene adhering to the fibre by blowing with steam. Without the occurrence of waste water, there is obtained a red dyeing which is rinsed clear and has the same fastness properties as a dyeing rinsed with an aqueous washing liquor.

Without the additives to the perchloroethylene after-treatment bath, a dyeing of poor fastness properties is obtained, since the dyestuff which is not bound by the fibre is not removed from the fabric.



## EXAMPLE 7

A polyacrylonitrile fabric is padded with an emulsion consisting of

10 parts of the dyestuff VI  
 11 parts of 85% formic acid  
 9 parts of 60% acetic acid  
 12 parts ethylene-cyanohydrin  
 8 parts glycerol monoacetate  
 8 parts methyl glycol acetate  
 4 parts nonylphenol decaethylene glycol ether  
 88 parts of water and  
 850 parts perchloroethylene

(liquor absorption 100%), dried at 100° C. for 1 minute and thermosolised at 200° C. for 1 minute.

The fabric then passes through 5 successive wash baths which have been heated to 50° C., each containing 5 parts of a mixture of

19.5 parts of the compound of the formula



1 part stearic acid

2 parts of the compound of the formula



0.5 parts oleyl alcohol heptadecaethylene glycol ether

3 parts of glacial acetic acid

19.5 parts isopropanol and

54.5 parts of water in 995 parts perchloroethylene,



(2) When 5 parts of the mixture are replaced with 5 parts of one of the following compounds of the Formulae a-g:



the time of residence amounting to 90 seconds in each bath and the liquor ratio of 1:50. The material is then rinsed with pure perchloroethylene, the solvent is separated and the adhering solvent residues are removed by blowing with steam. Without the occurrence of waste water, there is obtained a yellow dyeing which is rinsed clear.

If the compound of the formula



is replaced in the mixture with the same amount of the aminoxide of the formula



then the resultant dyeing is equally well rinsed.

The same good washing-out effect is achieved

(1) When the 19.5 parts of the compound of the formula



are replaced in the mixture described above with 19.5 parts of one of the following aminoxides of the Formulae a-e:



(4) When 5 parts of the mixture are replaced with 5 parts of a mixture consisting of

70 2.5 parts of a compound of the formula



(4) When 5 parts of the mixture are replaced with 5 parts of a mixture consisting of

70 2.5 parts of a compound of the formula



21

1.2 parts of a compound of the formula



0.6 part of a compound of the formula



0.4 part of a compound of the formula



22

5 parts of a compound of the formula



5 parts isopropanol

10 parts of water, and

980 parts perchloroethylene

10 and subsequently treated for 1 minute in a fresh rinsing bath at 55° C., which consists of  
990 parts perchloroethylene, and  
5 parts of 60% acetic acid.

15 After separating the rinsing liquor, the solvent adhering to the fabric is removed by blowing with steam. Without the occurrence of waste water, there is obtained a well-rinsed, clear yellow/red bicolour dyeing of good fastness properties.

If the 5 parts of the compound of the formula



25 are replaced with 5 parts of one of the ammonium compounds of the Formulae a-d



45 (d)  $[\text{---}[\text{CH}_3\text{---}(\text{CH}_2)_{7}\text{---CH=CH---}(\text{CH}_2)_7\text{---CONH---}(\text{CH}_2)_3\text{---N---}(\text{CH}_3)_3]^\oplus \text{CH}_3\text{OSO}_3^\ominus$   
or 5 parts of the tertiary amine of the formula



(a)



and  
0.3 part of a compound of the formula



and 5 parts isopropanol.

## EXAMPLE 8

A polyacrylonitrile/staple fibre mixed fabric (65:35) is padded with an emulsion consisting of

10 parts of the dyestuff I

10 parts of the dyestuff VII

60 parts urea

5 parts nonylphenol decaethylene glycol ether

15 parts sodium paraffin sulphonate

3 parts of glacial acetic acid

97 parts of water, and

800 parts perchloroethylene

(liquor absorption 80%), dried at 120° C. for 90 seconds and thermosolised at 200° C. for 90 seconds. The fabric is subsequently padded with an emulsion consisting of

20 parts sodium carbonate

100 parts of water

2 parts nonylphenol decaethylene glycol ether, and  
878 parts perchloroethylene

and steamed at 103° C. for 5 minutes.

The fabric is subsequently treated in a liquor ratio of 1:50 for 5 minutes in an after-treatment bath which has been heated to 55° C. and consists of

then the good washing-out effect and an equally satisfactory dyeing is achieved.

65

## EXAMPLE 9

A fabric of a polyester which can be dyed with basic dyestuffs is padded with an emulsion consisting of

70 10 parts of the dyestuff VIII

1 part oleic acid ethanolamide

2 parts nonylphenol decaethylene glycol ether

30 parts butyrolactone

21 parts urea

75 30 parts of 60% acetic acid

56 parts of water and  
850 parts perchloroethylene

with a liquor absorption of about 104%, dried at 100° C. for 90 seconds and thermosolised at 200° C. for 90 seconds.

The fabric is then treated in a liquor ratio of 1:50 for 3 minutes in an after-treatment bath at 50° C. consisting of

5 parts of the N,N-di-octadecyl-N,N-dimethyl ammonium salt of sulphated rapeseed oil

5 parts of water and  
990 parts perchloroethylene

and subsequently in an after-treatment bath consisting of

1 part of the N,N-di-octadecyl-N,N-dimethyl ammonium salt of sulphated rapeseed oil

1 part of water and  
998 parts perchloroethylene.

The material is subsequently rinsed with fresh perchloroethylene and after separating the solvent, the solvent residues adhering to the fibre are removed by blowing with steam. Without the occurrence of waste water, there is obtained a full blue dyeing which has the same fastness properties as a dyeing rinsed in water.

When the 5 parts in the first after-treatment bath and the 1 part in the second after-treatment bath, of N,N-di-octadecyl-N,N-dimethyl ammonium salt of sulphated rapeseed oil are replaced with 5 parts and 1 part, respectively, of a mixture of

3 parts of the compound of the formula



and

9 parts isopropanol,

then the same washing-out effect is achieved.

#### EXAMPLE 10

A mixed fabric (50:50) of a polyamide which can be dyed with basic dyestuffs and a polyamide which can be dyed with acidic dyestuffs is padded with an emulsion consisting of

10 parts of the dyestuff I

10 parts of the dyestuff IX

4 parts of the reaction product of 1 mol oleyl alcohol with 50 mol ethylene oxide

4 parts nonylphenol decaethylene glycol ether

3 parts of a mixture consisting of

20 parts of a compound of the formula



40 parts oleyl alcohol eicosethylene glycol ether and

40 parts ethyl hexanol

5 parts of 60% acetic acid

80 parts of water and

884 parts perchloroethylene

with a liquor absorption of 70%, dried at 80° C. for 1 minute and steamed at 105° C. for 3 minutes.

The fabric web then successively passes in a liquor ratio of 1:30 with a time of residence of 2 minutes each time through two after-treatment baths which are mechanically agitated and have been heated to 50° C. and which consist of

0.75 part of the N,N-di-octadecyl-N,N-dimethyl ammonium salt of sulphated rapeseed oil

0.75 parts of a compound of the formula



5 0.5 parts of a compound of the formula



10 1 part of the reaction product of 1 mol oleyl alcohol eicosethylene glycol ether and

5 parts of water in 980 parts perchloroethylene

and subsequently with a time of residence of 1 minute through a rinsing bath of pure perchloroethylene which has been heated to 50° C. After separating the rinsing liquor, the fabric is freed from the adhering perchloroethylene by blowing with steam. Without the occurrence of waste water, there is obtained a dyeing with a yellow-blue pattern of excellent fastness properties.

#### EXAMPLE 11

A Turkish towelling fabric of cotton is padded with an emulsion consisting of

25 40 parts of the dyestuff X

80 parts urea

98 parts of water

10 parts sodium bicarbonate

5 parts nonylphenol decaethylene glycol ether and

767 parts perchloroethylene,

dried at 140° C. for 1 minute and condensed at 150° C. for 3 minutes.

The fabric is subsequently after-treated in a liquor ratio of 1:40 for 3 minutes each time in two successive baths which have been heated to 50° C. and consists of

5 parts of a compound of the formula



40 5 parts of 60% acetic acid

10 parts of water and

980 parts perchloroethylene

and subsequently rinsed at the same temperature for 2 minutes with fresh perchloroethylene. After separating the rinsing liquor, the solvent residues are removed by blowing with steam. Without the occurrence of waste water, there is obtained a yellow dyeing which has been rinsed clear and has faultless fastness properties.

#### EXAMPLE 12

A polyacrylonitrile/cotton mixed fabric (50:50) is padded with an emulsion consisting of

55 9 parts of the dyestuff XI

26 parts of ethylene-cyanohydrin

15 parts formamide

2 parts nonylphenol decaethylene glycol ether

60 1 part oleic acid ethanolamide

60 parts urea

90 parts of water and

804 parts perchloroethylene

(liquor absorption 100%), dried at 80° C. for 90 seconds and thermosolised at 202° C. for 1 minute.

The fabric subsequently passes with a time of residence of 90 seconds each time through 6 successive after-treatment baths which have been heated to 50° C. and consist of

5 parts of the compound of the formula



15 parts of water and

75 980 parts perchloroethylene.

25

The material is then rinsed in pure perchloroethylene at 50° C., the rinsing liquor is separated and the fabric freed from the adhering solvent by blowing with steam. Without the occurrence of waste water, there is obtained a dyeing with a yellow/white effect which has been rinsed clear and has the same fastness properties as a dyeing after-treated with aqueous baths.

If the 5 parts of the compound of the formula



are replaced with 5 parts of the compound of the formula



then the resultant dyeing is rinsed equally clear.

#### EXAMPLE 13

A staple fibre fabric is padded with an emulsion consisting of

30 parts of the dyestuff XII  
4 parts nonylphenol pentadecethylene glycol ether  
80 parts urea  
10 parts sodium bicarbonate  
90 parts of water and  
786 parts perchloroethylene

(liquor absorption 80%), dried at 80° C. for 1 minute and steamed with overheated steam at 150° C. and normal pressure for 1 minute.

The fabric is subsequently after-treated in a liquor ratio of 1:50 for 2 minutes each time in 5 successive baths which have been heated to 55° C. and consisting of

1 part of the dyestuff XV

0.6 parts of the dyestuff VIII

7.5 parts urea

6.9 parts of water

15 parts of a mixture consisting of

12 parts of water

30 parts sodium paraffin sulphonate

2.5 parts sodium dodecyl-benzene sulphonate and  
17.5 parts of the sulphuric acid ester of a sperm oil alcohol,

as well as

3115 parts perchloroethylene.

54 parts of a mixture consisting of

0.6 parts sodium carbonate

10.4 parts of water

5 parts urea

32 parts perchloroethylene and

6 parts of a mixture consisting of

30 parts sodium paraffin sulphonate

2.5 parts sodium dodecyl-benzene sulphonate

17.5 parts of the sulphuric acid ester of a sperm oil alcohol

12 parts of water

25 are then added to the dyebath and the treatment is continued at 40° C. for 1 hour. The dyebath is subsequently heated to 110° C. within 20 minutes and the same temperature is maintained for 1 hour. The dyeing emulsion is then drained off, and the fabric rinsed with fresh perchloroethylene.

30 The fabric is then after-treated in a liquor ratio of 1:20 with a time of residence of 10 minutes with a bath which has been heated to 50° C. and consists of

5 parts of the compound of the formula



5 parts of a compound of the formula



5 parts isopropanol

5 parts of water

5 parts of 60% acetic acid and

985 parts perchloroethylene

and then rinsed with fresh perchloroethylene. After separating the rinsing liquor, the fabric is freed from the adhering solvent residues by blowing with steam. The resultant red dyeing has been rinsed clear and has the same fastness properties as a dyeing rinsed with an aqueous liquor.

If the compound of the formula



is replaced with 5 parts of the compound of the formula



or with 4 parts of a mixture of the two compounds, then the same good washing-out effect is achieved.

#### EXAMPLE 14

100 parts of a polyester/cotton mixed fabric (67:33) are printed in a pressure winding frame at 40° C. for 30 minutes with an emulsion consisting of

26

1 part of the dyestuff XV

0.6 parts of the dyestuff VIII

7.5 parts urea

6.9 parts of water

15 parts of a mixture consisting of

12 parts of water

30 parts sodium paraffin sulphonate

2.5 parts sodium dodecyl-benzene sulphonate and  
17.5 parts of the sulphuric acid ester of a sperm oil alcohol,

as well as

3115 parts perchloroethylene.

54 parts of a mixture consisting of

0.6 parts sodium carbonate

10.4 parts of water

5 parts urea

32 parts perchloroethylene and

6 parts of a mixture consisting of

30 parts sodium paraffin sulphonate

2.5 parts sodium dodecyl-benzene sulphonate

17.5 parts of the sulphuric acid ester of a sperm oil alcohol

12 parts of water

25 are then added to the dyebath and the treatment is continued at 40° C. for 1 hour. The dyebath is subsequently heated to 110° C. within 20 minutes and the same temperature is maintained for 1 hour. The dyeing emulsion is then drained off, and the fabric rinsed with fresh perchloroethylene.

30 The fabric is then after-treated in a liquor ratio of 1:20 with a time of residence of 10 minutes with a bath which has been heated to 50° C. and consists of

5 parts of the compound of the formula



5 parts of water

2 parts of 60% acetic acid and

988 parts perchloroethylene

45 The fabric is subsequently rinsed with pure perchloroethylene at 50° C. for 2 minutes. After separating the rinsing liquor, the fabric is freed from the adhering solvent by blowing with steam. There is obtained a red/blue bicolour dyeing which has the same fastness properties as a dyeing washed with aqueous wash baths.

50

#### EXAMPLE 15

A cotton fabric is padded with an emulsion consisting of

40 parts of the dyestuff XIV

3 parts nonylphenol decaethylene glycol ether

60 parts urea

10 parts sodium carbonate

100 parts of water and

787 parts perchloroethylene

60 (liquor absorption 80%), dried at 80° C. for 1 minute and steamed at 102° C. for 5 minutes.

The fabric is subsequently after-treated in a liquor ratio of 1:50 with a time of residence of 2 minutes each time in 3 successive baths which have been heated to 55° C. and consist of

5 parts of the aminoxide of the formula



70 10 parts of water and

985 parts perchloroethylene.

The fabric is then rinsed with pure perchloroethylene at 55° C., for 2 minutes. After separating the rinsing liquor,

the fabric is freed from the adhering perchloroethylene residues in an air current. A clear yellow dyeing is obtained without the occurrence of waste water.

## EXAMPLE 16

A polyester/cotton mixed fabric (65:35) is padded with an emulsion consisting of

12 parts of the dyestuff XVI

2 parts nonylphenol decaethylene glycol ether

1 part oleic acid ethanol amide

20 parts of the dyestuff VII

60 parts urea

8 parts sodium bicarbonate

97 parts of water and

800 parts perchloroethylene

(liquor absorption 80%), dried at 120° C. for 60 seconds and thermosolised at 180° for 60 seconds.

The fabric then passes through 5 successive washing aggregates which operate according to the counter-current principle and contains a solution at 55° C. consisting of

5 parts of the compound of the formula



5 parts of water and

990 parts perchloroethylene.

The liquor ratio for the after-treatment amounts to 1:100.

The fabric is subsequently rinsed with a mixture at 55° C. consisting of

990 parts perchloroethylene

5 parts of 60% acetic acid and

5 parts of water.

After separating the rinsing liquor, the fabric is freed from the adhering solvent residues by blowing with air. Without the occurrence of waste water there is obtained a clear dyeing with a red/yellow pattern which has the same fastness properties as a dyeing after-treated with aqueous liquors.

## EXAMPLE 17

A polyester/staple fibre mixed fabric (70:30) is padded with an emulsion consisting of

20 parts of the dyestuff XVI

15 parts of the dyestuff XIV

50 parts urea

70 parts nonylphenol hexaethylene glycol ether

5 parts sodium bicarbonate

60 parts of water and

780 parts perchloroethylene

(liquor absorption 80%), dried at 120° C. for 90 seconds and thermosolised at 180° C. for 90 seconds.

The fabric is subsequently after-treated in a liquor ratio of 1:50 for 5 minutes in bath at 55° C. consisting of

5 parts of the compound of the formula



10 parts of 30% acetic acid and

985 parts perchloroethylene

and then rinsed with pure perchloroethylene at 55° C. for 1 minute. After separating the rinsing liquor, the fabric is freed from the adhering solvent residues by blowing with hot air. The resultant clear yellow dyeing is well washed out.

The same good washing-out effect is achieved when the 5 parts of the compound of the formula



are replaced with

(a) 5 parts of a mixture of equal parts of the compound of the formula



and oleic acid or

(b) 5 parts of a mixture of equal parts of the compound of the formula



and the compound of the formula



or

(c) 5 parts of a mixture of equal parts of the compound of the formula



and the compound of the formula



or

(d) 5 parts of the N,N-diocadecyl-N,N-dimethyl ammonium salt of sulphated rapeseed oil or

(e) 5 parts of a mixture of

18.5 parts of the compounds of the formula



17.5 parts of the compound of the formula



and

8 parts isopropanol or

(f) 5 parts of a mixture of

18 parts of the compound of the formula



17.5 parts of the compound of the formula



and

8 parts isopropanol

## EXAMPLE 18

A fabric of polyhexamethylene-diamine adipate is padded with an emulsion consisting of

20 parts of the 1:2 chromium complexes of the dyestuff XVII

3 parts nonylphenol decaethylene glycol ether

80 parts urea

100 parts of water and

797 parts perchloroethylene

(liquor absorption 80%), dried at 80° C. for 90 seconds and thermosolised at 210° C. for 1 minute.

The fabric then passes in a liquor ratio of 1:50 and with a time of residence of 2 minutes each time through

29

4 successive after-treatment baths which have been heated to 55° C. and consist of  
 6 parts N,N-di-eicosyl-N,N-dimethyl ammonium bromide  
 6 parts of water  
 1 part octadecyl alcohol heptadecaethylene glycol ether and  
 987 parts perchloroethylene.

The fabric web then passes with a time of residence of 1 minute through a rinsing bath of pure perchloroethylene which has been heated to 50° C. After separating the rinsing liquor, the fabric is freed from the adhering perchloroethylene residues by blowing with hot air. The resultant red dyeing is rinsed clear without the occurrence of waste water and has the same fastness properties as a dyeing rinsed with water.

## EXAMPLE 19

A cellulose/poly- $\epsilon$ -caprolactam mixed fabric (50:50) is padded with an emulsion consisting of

20 parts of the dyestuff VII  
 20 parts of the 1:2 chromium complex of the dyestuff XVIII

3 parts nonylphenol decaethylene glycol ether

6 parts sodium bicarbonate

80 parts urea

100 parts of water and

771 parts perchloroethylene

(liquor absorption 40%), dried at 100° C. for 1 minute and thermosolised at 192° C. for 60 seconds.

The fabric web then successively passes in a liquor ratio of 1:50 and with a time of residence of 2 minutes each time through 4 after-treatment baths which are

30

mechanically agitated and have been heated to 55° C. and consist of

4 parts of the compound of the formula



1 part of the compound of the formula



20 1 part of the compound of the formula



7 parts of 30% acetic acid and

25 987 parts perchloroethylene

and subsequently with a time of residence of 1 minute through a rinsing bath of pure perchloroethylene which has been heated to 55° C. After separating the rinsing liquor, the fabric is freed from the adhering perchloroethylene residues by blowing with air and steam. The resultant bicolour dyeing has been rinsed clear without the occurrence of waste water and has the same fastness properties as a dyeing rinsed with water.

## CONSTITUTIONS OF THE DYESTUFFS I-XVIII USED IN THE EXAMPLES

| Number | Constitution                                                                                                                                                                                                                                  |
|--------|-----------------------------------------------------------------------------------------------------------------------------------------------------------------------------------------------------------------------------------------------|
| I      | $[\text{CH}_3-\text{C}_6\text{H}_4-\text{N}^+(\text{CH}_3)_2-\text{CH}=\text{CH}-\text{N}(\text{C}_6\text{H}_4-\text{CH}_2-\text{CH}_2-\text{H}_2)-\text{CH}_2-\text{CH}_2-\text{H}_2] \text{Cl}^-$                                           |
| II     | $[\text{O}_2\text{N}-\text{C}_6\text{H}_4-\text{Cl}-\text{N}=\text{N}-\text{C}_6\text{H}_4-\text{N}(\text{C}_2\text{H}_5)_2-\text{CH}_2-\text{CH}_2-\text{N}^+(\text{CH}_2-\text{CH}_2-\text{N}(\text{CH}_2)_3)_2] \text{CH}_3\text{OSO}_3^-$ |
| III    | $[\text{C}_6\text{H}_3(\text{O})_2-\text{C}_6\text{H}_4-\text{NH}-\text{CH}_2-\text{CH}_2-\text{CH}_2-\text{N}^+(\text{CH}_2-\text{CH}_2-\text{N}(\text{CH}_2)_3)_2] \text{CH}_3\text{OSO}_3^-$                                               |
| IV     | $[(\text{C}_2\text{H}_5)_2-\text{N}-\text{C}_6\text{H}_4-\text{O}-\text{C}_6\text{H}_4-\text{N}^+(\text{C}_2\text{H}_5)_2-\text{O}-\text{C}_2\text{H}_5] \text{Cl}^-$                                                                         |
| V      | $[\text{O}_2\text{N}-\text{C}_6\text{H}_4-\text{N}=\text{N}-\text{C}_6\text{H}_4-\text{N}(\text{C}_2\text{H}_5)_2-\text{CH}_2-\text{CH}_2-\text{N}^+(\text{CH}_2-\text{CH}_2-\text{N}(\text{CH}_2)_3)_2] \text{CH}_3\text{OSO}_3^-$           |
| VI     | $[\text{CH}_3-\text{C}_6\text{H}_4-\text{N}^+(\text{CH}_3)_2-\text{CH}=\text{CH}-\text{C}_6\text{H}_4-\text{N}(\text{CH}_2-\text{CH}_2-\text{Cl})_2] \text{Cl}^-$                                                                             |

## CONSTITUTIONS OF THE DYESTUFFS I-XVIII USED IN THE EXAMPLES.—Continued

Number Constitution

VII.....



VIII.....



IX.....



X.....



XI.....



XII.....



XIII.....



XVI.....



| Number     | Constitution |
|------------|--------------|
| XV.....    |              |
| XVI.....   |              |
| XVII.....  |              |
| XVIII..... |              |

We claim:

1. In the process of dyeing or printing textile materials comprising the steps of (A) impregnating the textile material with chlorinated hydrocarbon/water dyestuff emulsions, the aqueous phase of which contains a solution of water-soluble dyestuff, (B) heat treating the textile material to fix the dyestuff; (C) rinsing the textile material to remove dyestuff which is non-fixed; the improvement comprising conducting the rinsing step (C) with a solution consisting essentially of an aliphatic chlorinated hydrocarbon solvent and dissolved therein interface-active compound means for rendering the dyestuff which was not fixed in step (B) dispersible or soluble in said chlorinated hydrocarbon solvent, said interface-active compound being interface-active in said chlorinated hydrocarbon solvent.

2. The process of claim 1 in which the interface-active compound is present in amounts of 0.02–2% by weight, based on the weight of the aliphatic chlorinated hydrocarbon.

3. The process of claim 1 in which the aliphatic chlorinated hydrocarbon solution contains 0.02–4% by weight of water based on the weight of aliphatic chlorinated hydrocarbon.

4. The process of claim 3 in which the aliphatic chlorinated hydrocarbon solution contains 0.001–2% by weight of non-ionic emulsifier based on the weight of aliphatic chlorinated hydrocarbon.

5. The process of claim 1 in which the aliphatic chlorinated hydrocarbon solution contains 0.001–8% by weight of water-miscible organic solvent based on the weight of the aliphatic chlorinated hydrocarbon.

6. The process of claim 1 in which the interface-active compound is an onium compound of the formula



in which  
A is nitrogen or phosphorus;  
40 R<sub>1</sub> is an alkyl, alkenyl or aralkyl radical of 12–28 carbon atoms or one of the aforesaid radicals containing oxygen, sulfur or nitrogen;  
R<sub>2</sub> and R<sub>3</sub> independently of one another, are unsubstituted or substituted alkyl, alkenyl, or aralkyl radicals which contain 1–28 carbon atoms or one of the aforesaid radicals containing oxygen, sulfur or nitrogen;  
45 R<sub>4</sub> is substituted or unsubstituted C<sub>1</sub>–C<sub>14</sub>-alkyl, C<sub>1</sub>–C<sub>14</sub>-alkenyl, cycloalkyl or aralkyl or together with R<sub>3</sub> forms a non-aromatic 5- or 6-membered heterocycle; with the proviso that the sum of carbon atoms in R<sub>1</sub>, R<sub>2</sub>, R<sub>3</sub>, and R<sub>4</sub> is 20 to 60; and  
X<sup>–</sup> is an anion.

7. The process of claim 1 in which the interface-active compound is a quaternary ammonium compound of the formula



60 in which  
R<sub>1</sub> is an alkyl, alkenyl or aralkyl radical of 12–28 carbons, or one of the aforesaid radicals containing oxygen, sulfur or nitrogen;  
R<sub>2</sub> is an unsubstituted or substituted alkyl, alkenyl or aralkyl radical of 1–28 carbon atoms or one of the aforesaid radicals containing oxygen, sulfur or nitrogen;  
65 R<sub>3</sub> is an unsubstituted or substituted C<sub>1</sub>–C<sub>14</sub>-alkyl, C<sub>1</sub>–C<sub>14</sub>-alkenyl, cycloalkyl or aralkyl radical, or together with R<sub>3</sub> forms a non-aromatic 5- or 6-membered heterocycle;  
R<sub>4</sub> is an alkylene radical which contains 1–8 carbon atoms, a C<sub>1</sub>–C<sub>8</sub>-alkylene which contains oxygen atoms or 1,4-bis-methylene-benzene radical; with the proviso that the sum of carbon atoms in R<sub>1</sub>, R<sub>2</sub>, R<sub>3</sub> and R<sub>4</sub> and Z is 20 to 60; and

35

$Y^-$  is the anionic grouping  $-\text{SO}_3^-$ ,  $-\text{OSO}_3^-$ ,  $-\text{S}-\text{SO}_3^-$ ,  $-\text{OPO}_3^{2-}$ , or  $-\text{COO}^-$ .

8. The process of claim 1 in which the interface-active compound is an amine of the formula



in which

$\text{R}_1$  is an alkyl, alkenyl or aralkyl radical of 12-28 carbon atoms or one of the aforesaid radicals containing oxygen, sulfur or nitrogen;

$\text{R}_2$  is an unsubstituted or substituted  $\text{C}_1-\text{C}_{14}$ -alkyl,  $\text{C}_1-\text{C}_{14}$ -alkenyl, cycloalkyl or aralkyl radical;

$\text{R}_5$  is hydrogen, an unsubstituted or substituted alkyl, alkenyl or aralkyl radical of 1-28 carbon atoms or one of the aforesaid radicals containing oxygen, sulfur or nitrogen, or  $\text{R}_5$  together with  $\text{R}_4$  forms a 5- or 6-membered non-aromatic heterocycle; with the proviso that the sum of carbon in  $\text{R}_1$ ,  $\text{R}_4$  and  $\text{R}_5$  is 20 to 60.

9. The process of claim 1 in which the interface-active compound is an aminoxide of the formula



in which

$\text{R}_1$  is an alkyl, alkenyl or aralkyl radical of 12-28 carbon atoms or one of the aforesaid radicals containing oxygen, sulfur or nitrogen;

$\text{R}_3$  is an unsubstituted or substituted alkyl, alkenyl or aralkyl radical of 1-28 carbon atoms or one of the aforesaid radicals containing oxygen, sulfur or nitrogen; and

$\text{R}_4$  is an unsubstituted or substituted  $\text{C}_1-\text{C}_{14}$ -alkyl, or  $\text{C}_1-\text{C}_{14}$ -alkenyl, cycloalkyl or aralkyl radical or together with  $\text{R}_3$  forms a non-aromatic 5- or 6-membered heterocycle; with proviso that the sum of carbon atoms in  $\text{R}_1$ ,  $\text{R}_3$  and  $\text{R}_4$  is 20 to 60.

10. The process of claim 1 in which said chlorinated

hydrocarbon/water emulsion contains a water-soluble dyestuff in the aqueous phase and a chlorinated hydrocarbon soluble dyestuff in the chlorinated hydrocarbon phase.

5 11. The process of claim 1 in which the aliphatic chlorinated hydrocarbon solution contains a compound selected from the group consisting of 0.01% to 1.0% by weight of acetic acid, 0.01% to 0.5% by weight of monoethanolamine 0.01% to 0.5% by weight of diethanolamine and 0.01% to 0.5% by weight of triethanolamine.

12. In the process of dyeing textile materials comprising the steps of (A) exhaustion dyeing a textile material with chlorinated hydrocarbon/water dyestuff emulsions, the aqueous phase of which contains a solution of water-soluble dyestuff; and (B) rinsing to remove excess dyestuff, the improvement comprising conducting the rinsing step (B) with a solution consisting essentially of aliphatic chlorinated hydrocarbon solvent and dissolved therein interface-active compound means for rendering the excess dyestuff dispersible or soluble in said chlorinated hydrocarbon solvent, said interface-active compound being interface-active in said chlorinated hydrocarbon solvent.

#### References Cited

##### UNITED STATES PATENTS

|           |         |                      |         |
|-----------|---------|----------------------|---------|
| 3,523,749 | 8/1970  | MacLeod et al. ----- | 8-94 X  |
| 2,828,180 | 3/1958  | Sertorio -----       | 8-62    |
| 3,510,243 | 5/1970  | Seuret et al. -----  | 8-174 X |
| 3,370,330 | 2/1968  | Sieber -----         | 26-19   |
| 2,274,751 | 3/1942  | Sowter et al. -----  | 8-173   |
| 3,473,175 | 10/1969 | Sieber -----         | 8-158   |

##### OTHER REFERENCES

35 WAS White, Amer. Dyestuff Reporter, July 31, 1967, pp. 18-24.

LEON D. ROSDOL, Primary Examiner

T. J. HERBERT, JR., Assistant Examiner

U.S. CL. X.R.

8-94, 169, 171, 172, 173

UNITED STATES PATENT OFFICE  
CERTIFICATE OF CORRECTION

PATENT NO. : 3,764,262

DATED : October 9, 1973

INVENTOR(S) : DIETRICH HILDEBRAND ET AL.

It is certified that error appears in the above-identified patent and that said Letters Patent are hereby corrected as shown below:

| <u>COLUMN</u> | <u>LINE</u> | <u>ERROR</u>                                                                                                                   |
|---------------|-------------|--------------------------------------------------------------------------------------------------------------------------------|
| 2             | 36          | "-SO-SO <sub>3</sub> -" should read<br>--- -S-SO <sub>3</sub> - ---                                                            |
| 5             | 57          | "CH <sub>2</sub> CH <sub>2</sub> -CN" should read<br>--- CH <sub>2</sub> -CH <sub>2</sub> -CN ---                              |
| 5             | 62          | "CH <sub>2</sub> CH <sub>3</sub> " should read --- CH <sub>2</sub> -CH <sub>3</sub> ---                                        |
| 5             | 66          | "CH <sub>2</sub> CH <sub>2</sub> -Cl" should read<br>--- CH <sub>2</sub> -CH <sub>2</sub> -Cl ---                              |
| 5             | 69          | "CH <sub>2</sub> CH <sub>2</sub> -OSO <sub>3</sub> " should read<br>--- CH <sub>2</sub> -CH <sub>2</sub> -OSO <sub>3</sub> --- |
| 5             | 73          | "CH <sub>2</sub> -CH <sub>2</sub> OPO <sub>3</sub> " should read<br>--- CH <sub>2</sub> -CH <sub>2</sub> -OPO <sub>3</sub> --- |

Signed and Sealed this

ninth Day of September 1975

[SEAL]

Attest:

RUTH C. MASON  
Attesting Officer

C. MARSHALL DANN  
Commissioner of Patents and Trademarks

UNITED STATES PATENT OFFICE  
CERTIFICATE OF CORRECTION

PATENT NO. : 3,764,262

DATED : October 9, 1973

INVENTOR(S) : DIETRICH HILDEBRAND ET AL.

It is certified that error appears in the above-identified patent and that said Letters Patent are hereby corrected as shown below:

| <u>COLUMN</u> | <u>LINE</u> | <u>ERROR</u>                                                                                                   |
|---------------|-------------|----------------------------------------------------------------------------------------------------------------|
| 6             | 55          | " $\text{CH}_2$ " should read --- $\text{CH}_3$ ---                                                            |
| 9             | 49          | "diisobdutyl-" should read<br>--- diisobutyl- ---                                                              |
| 13            | 14          | "wthout" should read --- without ---                                                                           |
| 15            | 23          | " $(\text{CH}_2)_{20}$ " should read<br>--- $(\text{CH}_2)_{10}$ ---                                           |
| 15            | 26          | " $\text{CH}_3$ " should read<br>$\overset{\circ}{\text{S}}$<br>--- $\overset{\circ}{\text{S}}\text{CH}_3$ --- |
| 15            | 33          | " $\text{CH}_3$ " should read<br>--- $\text{CH}_2$ ---                                                         |
| 15            | 35          | " $\text{CH}_2$ " should read --- $\text{CH}_3$ ---                                                            |
| 17            | 33          | " $-\text{CH}=(\text{CH}_2)_7$ " should read<br>--- $\text{CH}=\text{CH}-(\text{CH}_2)_7$ ---                  |

Signed and Sealed this

ninth Day of September 1975

[SEAL]

Attest:

RUTH C. MASON  
Attesting Officer

C. MARSHALL DANN  
Commissioner of Patents and Trademarks

**UNITED STATES PATENT OFFICE**  
**CERTIFICATE OF CORRECTION**

PATENT NO. : 3,764,262

DATED : October 9, 1973

INVENTOR(S) : DIETRICH HILDEBRAND ET AL.

It is certified that error appears in the above-identified patent and that said Letters Patent are hereby corrected as shown below:

| <u>COLUMN</u> | <u>LINE</u> | <u>ERROR</u>                                                                                                                            |
|---------------|-------------|-----------------------------------------------------------------------------------------------------------------------------------------|
| 17            | 57          | "-S <sub>3</sub> O <sub>3</sub> <sup>⊖</sup> " should read<br>--- -SO <sub>3</sub> <sup>⊖</sup> ---                                     |
| 20            | 40          | " ] <sup>⊕</sup> CH <sub>3</sub> OSO <sub>3</sub> " should read<br>--- ] <sup>⊕</sup> CH <sub>3</sub> OSO <sub>3</sub> <sup>⊖</sup> --- |
| 20            | 47          | " \ " <sup>CH<sub>2</sub></sup> should read<br>--- \ " <sup>CH<sub>3</sub></sup> ---                                                    |
| 20            | 60          | After the formula insert --- and ---                                                                                                    |
| 21            | 3           | " ] <sup>⊖</sup> Cl <sup>⊖</sup> " should read<br>--- ] <sup>⊕</sup> Cl <sup>⊖</sup> ---                                                |
| 23            | 29          | "octadecyl-" should read<br>--- octadecyl- ---                                                                                          |

**Signed and Sealed this**

*ninth Day of September 1975*

[SEAL]

Attest:

**RUTH C. MASON**  
*Attesting Officer*

**C. MARSHALL DANN**  
*Commissioner of Patents and Trademarks*

UNITED STATES PATENT OFFICE  
CERTIFICATE OF CORRECTION

PATENT NO. : 3,764,262

DATED : October 9, 1973

INVENTOR(S) : DIETRICH HILDEBRAND ET AL.

It is certified that error appears in the above-identified patent and that said Letters Patent are hereby corrected as shown below:

| <u>COLUMN</u> | <u>LINE</u>               | <u>ERROR</u>                                                                                                                                                        |
|---------------|---------------------------|---------------------------------------------------------------------------------------------------------------------------------------------------------------------|
| 25            | 58                        | "CH <sub>3</sub> " should read --- CH <sub>3</sub> ---<br>N                                                                                                         |
| 26            | 69                        | "(CH <sub>2</sub> ) <sub>3</sub> ]" should read<br>--- (CH <sub>2</sub> ) <sub>3</sub> ---<br>[ ]<br>" ] Cl <sup>⊖</sup> " should read<br>--- ] Cl <sup>⊖</sup> --- |
| 28            | 18                        |                                                                                                                                                                     |
| 30            | No. III<br>in the formula | "CH <sub>3</sub> OSO <sup>⊖</sup> " should read<br>--- CH <sub>3</sub> OSO <sub>3</sub> <sup>⊖</sup> ---                                                            |
| 34            | 56                        | "R <sub>1</sub> <sup>+</sup> " should read<br>--- R <sub>1</sub> <sup>+</sup> ---                                                                                   |

Signed and Sealed this

ninth Day of September 1975

[SEAL]

Attest:

RUTH C. MASON  
Attesting Officer

C. MARSHALL DANN  
Commissioner of Patents and Trademarks